

Jan. 6, 1942.

C. T. DICKEY

2,268,703

PROCESS FOR MAKING BLANKS

Filed Dec. 5, 1939



Fig. 1.



Fig. 2.



Fig. 3.



Fig. 4.



Fig. 5.



Fig. 6.



Fig. 7.



Fig. 8.



Fig. 9.

INVENTOR.

Charles Thomas Dickey  
BY *Turner, Wisconsin*  
*for inventor*

## UNITED STATES PATENT OFFICE

2,268,703

## PROCESS FOR MAKING BLANKS

Charles Thomas Dickey, Elizabeth, N. J.

Application December 5, 1939, Serial No. 307,611

9 Claims. (Cl. 18—47.5)

This invention relates to process for making blanks having peripheral frictional properties applicable to, and used for, engaging a travelling fabric surface.

As is well-known to those working in textile operations, fabric-engaging rolls heretofore employed, such as those used in loom temples, are prone to quickly wear and become smooth due to constant tension and friction. As they become smooth, they progressively lose their efficiency for gripping fabric surfaces and must be often replaced, these frequent replacements being both time-consuming and costly.

It is one object of this invention to describe the method of manufacture of a roughly cylindrical and satisfactory blank containing therein immovably fixed plurality of fiber ends outwardly - projecting or outwardly - protruding therefrom.

Another object is to produce a cloth-engaging blank which retains its effective initial gripping surface substantially unimpaired for an indefinite time.

It is a further object to disclose a process for making such blanks which is simple, economical and expeditious, and wherein the initially satisfactory degree of frictional contact with textile surface is not materially diminished by continued usage over a long period.

Other objects will appear from the description and accompanying drawing, and particularly pointed out in the claims.

In the drawing and illustrative examples herein shown and described, the process of my invention as applied to a specific product—a temple roll—is as follows:

Figure 1 is a vertical cross-section showing a device adapted for the impregnation of blank material.

Figure 2 is a vertical cross-section of a portion of a punch adapted to form one of the blank units of my process.

Figure 3 is a face view of a unit employed in my process.

Figure 4 is a side view of the device of Figure 3.

Figure 5 is a vertical cross-section of a plurality of blank units positioned upon a supporting rod or mandrel.

Figure 6 is a vertical cross-section of the device of Figure 5 positioned within a molding press.

Figure 7 is a section through the line 7—7 of Figure 6 with the two elements of the molding press spaced from each other.

Figure 8 is the Figure 7 with the two elements of the molding press in molding position.

Figure 9 shows one method of the roughening or abrading process applied to the molded form of my device.

This drawing of one form of my invention is adapted to be used in connection with the usual type of temple, wherein two rolls are rotatively mounted. The temples are arranged in pairs, one at each side of the loom, and may be termed right-handed and left-handed since their function is to laterally stretch the cloth being woven to the right and left side of the loom.

The following is one process for producing the rolls of my invention, although it is evident that other steps of process may be employed without going beyond the scope of my invention, and is illustrated in the accompanying drawing and is described in some detail in order that the production of my devices may be clearly understood.

I take fabric, preferably strong fabric such as cotton duck, drill, or canvas, and saturate or impregnate the same with a suitable medium which is solid at normal room temperatures, such as a natural or synthetic resin or resin-like composition, or compound containing the same or its equivalent, preferably of a thermoplastic body or a body made thermoplastic by addition thereto.

The thermoplastic body or resin or resin-like material may be applied to the fabric in the heated state if the viscosity, wetting power, and other characteristics are suitable, or may be applied in solution or suspension form using an appropriate solvent, solvent composition, or thermoplasticizing component, volatile solvent being afterwards removed, as by evaporation.

Or the fabric may be coated on one or both sides, or may be thoroughly impregnated or saturated at room or elevated temperature, as by a dipping process. The method of application of the thermoplastic composition is immaterial, inasmuch as the prime object is to partially or completely impregnate fabrics in a suitable manner.

By thermoplastic composition as used herein is to be understood as including suitable natural or synthetic resins and resinous bodies or compositions containing the same, which are susceptible to heat-fusion and cold-hardening a plurality of times. This would embrace cellulose derivatives as cellulose esters (nitrate, acetate, acetopropionate, acetobutyrate, and the like) of varying degree of esterification; the cellulose ethers (as methyl, ethyl, benzyl ethyl-

benzyl ethers) of varying degrees of etherification; cellulose ester-ethers (as methylcellulose acetate), and physical admixtures of the preceding one with the other, the degree of thermoplasticity being heightened by addition thereto suitable plasticizing agents, depending upon the properties desired in the finished blank, especially as to permanent thermoplasticity in the finished blank. Flexilizers, solvents, or non-solvents may be incorporated to give an initial viscosity or for other purposes.

I take one or more sheets of suitable or dissimilar fabric 10 and pass it through the thermoplastic material 11 in a flowable state in a container 12, the idlers 13 and 13' squeezing excess material from the fabric 10 and allowing it to flow back into the container 12. The sheet 10 is then allowed to cool, dry, and harden; in which condition it is comparatively stiff, and it is then subjected to a punching process in order to produce a plurality of disks or washers adapted for the formation of my roll.

One form for the production of such disks is shown in Figure 2. This punch contains the two vertically movable punches 14 and 15, punch 14 being hollow and punch 15 having a centrally positioned opening 15' for the passage of punch 14. A plurality of sheets of prepared fabric 10, 10 is placed between the punches 14 and 15, punch 14 is moved downwardly, punch 15 is moved upwardly, and a disk or washer 16 having a central opening 16' is thus punched out of each sheet 10, the central cut-out portions of each sheet 10 being forced downwardly through the opening 15' of the punch 15 and thus removed from the device. It is desirable that the outside diameter of the washers 16, 16 be slightly greater than the outside diameter of the roll to be produced. It is evident that other means may be employed for the production of these disks.

A plurality of these disks or washers 16 are then placed upon a mandrel 7 as shown in Figure 5, which may be of a material such as wood, iron, steel, wood pulp, or the like of desired length and diameter.

If no central member is desired in the finished product, the washers may be assembled on a metal or other mandrel, the latter being subsequently removed from the compacted and agglutinated washers. If a central core or shaft is desired, the washers may be assembled on such core or shaft, and left on the same after the compacting operation has been completed.

After the desired number of washers 16, 16 have been placed on the mandrel or hollow shaft 17, they are subjected to pressure, or heat and pressure, as in a molding press, for a suitable length of time depending upon the degree of thermoplasticity of the body used.

As heat or heat and pressure is applied, the thermoplastic composition tends to liquify and uniformly flows in and around the fibers and fiber interstices of the textile, thereby welding the fiber washers into a continuous unitary-appearing mass.

One method of performing this step in the production of the rolls of my invention is shown in Figures 6, 7, and 8.

The mandrel 17 with its plurality of washers 16, 16 is placed between the upper member 18 and the lower member 19 of a press adapted to be heated by any convenient means (not shown), the inner face of the two press members 18 and 19 being formed into alternating ridges 20 and

grooves 21 to form a helix thus producing a surface to the finished roll adapted to perform its function of putting lateral tension on the cloth treated thereby.

5 The two heated members 18 and 19 are then brought together as shown in Figure 8, thus molding the outer face of the thus produced roll into a helical surface as shown. The pressure, or heat and pressure, is then released, the roll allowed to solidify by cooling, and is finally removed from the press. The mandrel 17 may be removed either at this time or afterward.

It will be noted that the fabric threads are so arranged in the finished mass that their long 15 axes are perpendicular to the long axis of the completed unit. Thus it is possible to have a large proportion of the ends of the fabric threads 20 protruding or projecting outwardly from the curved surface of the cylindrical blank, and upon this fact depends in a large measure the novelty and efficiency of the completed blank for many 25 purposes. It is highly important that a multiplicity of these fiber ends shall be projecting outwardly, that they may frictionally engage a cloth or other surface passing tangentially to the blank as it revolves.

I am aware that patents have issued for blanks or rolls made by impregnating fabric with an initially plastic or thermoplastic substance. In one of 30 them for instance, a fabric tube open at both ends is filled and expanded while the ends are held tight, by a plastic substance which is allowed to harden therein. The result is a fabric in roll form impregnated with plastic.

However in this, the finished roll has most of its 35 threads roughly parallel to the long axis of the roll, and the remaining threads lie in a plane concentric to the outer curved surface of the roll. Also as soon as the fabric wears through by friction in use, the roll is useless for frictional gripping purposes, as there is no fabric.

The process of my invention is in direct contrast to methods like the above in that the practice of my invention results in the formation of a 45 roll wherein the fabric planes are perpendicular to the long axis of the roll, and the fiber ends project outwardly from the surface of the roll to be used, thus constituting a frictional-gripping member, wherein wear does not materially diminish 50 the evenness of friction.

The compacted blanks after formation may be placed in a mold and furrowed, grooved, spirally channelled or otherwise altered in external configuration by means of pressure or pressure and heat.

55 If the finished blank is to be of other than cylindrical shape with a substantially smooth surface however, it is simpler that this result be accomplished in the previously described molding step. That is, if there is desired (say) helicoidally grooved form in the finished blank, a mold so shaped as to produce the grooves would be indicated in the compacting operation. An example of such a roll is shown in Fig. 6.

In the molding step, the thermoplastic binder usually flows closely to the mold surface, especially where sufficient pressure is exerted, so that the blank as it is removed from the mold has a smooth surface. In order to expose the fiber ends, it is desirable to submit the blank in this condition to some kind of a roughening or abrading treatment, without which the process would result in the formation of a member substantially valueless from a gripping standpoint, as the available

and outwardly-projecting fiber ends would not produce to induce the essential gripping effect.

For this step, I have found that grinding wheels give satisfactory results.

The speed of the wheel should be adjusted to suit the individual thermoplastic substance, and this is usually critical. If the speed is too high, frictional heat generated by the revolving wheel against the blank, intumesces or softens the thermoplastic and makes gummy, therefore difficult to handle, and leading to unsatisfactory results.

On the other hand, if the speed of rotation of the wheel is too low, the thermoplastic binder, instead of being smoothly rubbed off—that is, instead of being removed in minute particles, is removed in irregular and comparatively large aggregates, or in other words, is "chipped off," thus leaving the surface too irregular for satisfactory use.

Thus it is seen that in order to accomplish the abrading or roughening operation satisfactorily, which is in such manner that the maximum of fiber ends may be exposed, too much frictional heat tends to the production of an unworkable surface consistency, and the recurrent re-fusing of the thermoplastic mass, whereas too little frictional heat permits of insufficient softening of the bonding medium and leads to dislodgement of comparatively large particles from the surface.

It is apparent that in the latter case, dislodging of the aggregates also ruptures the threads, especially the fine counts of rayon threads thus causing the fiber ends to be removed, and this result diminishes or eliminates one of the chief advantages of the process, that of making a suitable blank with outwardly-projecting fiber ends. One method of producing this result is shown in Figure 9, in which the roughing roll, or cylinder, 20 supported on the shaft 21 is revolved with its surface in contact with the outer surface of the roll of my invention produced as previously described.

In this connection it should be noted that a substance which is not thermoplastic such as a thermosetting synthetic resin, as of the Bakelite type, or of rubber, will not become sufficiently plastic in the grinding operation to prevent the fiber rupturing above described from occurring.

As one method of carrying out my invention, I may take four pounds avoirdupois of 10 ounce duck which has or has not been woven with a proportion of asbestos fiber, and permeate or impregnate it with a solution of a thermoplastic synthetic resin, as of the vinol type, in a volatile solvent or solvent combination. The concentration of the solution is so adjusted that good flowability with minimum use of solvent is attained at the working temperature. After suitable impregnation the major portion of the solvent is removed by evaporation, the impregnated fabric then weighing about six pounds eleven ounces avoirdupois. From this sheet a plurality of washer-like members is cut, one of which is shown in Figs. 3 and 4, and then aligned over a mandrel and the assembly thus formed subjected to a pre-warming operation if desired, then to pressure, or heat and pressure in a suitable mold for a length of time which practice has indicated is optimum and most economical. In the above example, a temperature of about 60° centigrade and pressure of about 2000 pounds per square inch for about three minutes is sufficient.

The mold is then preferably cooled to about 35° C. or lower, and the blank removed.

Subsequently the extruded thermoplastic is

abraded off to expose the outwardly-projecting fiber ends.

In an alternative method, woven fiber sheets, either of cellulose matter or cellulose and inorganic matter as asbestos fibers, may be impregnated as in the previous example, using a cellulose derivative as a cellulose ester or ether, specifically highly etherified ethyl- or benzyl-cellulose or mixtures of the same, with or without solvents, non-solvents and/or thermoplasticizing bodies, depending in a large measure upon the relative thermoplasticity of the cellulose derivative employed.

A plurality of impregnated fiber sheets is then stacked one upon the other to a thickness somewhat greater than the length desired in the finished blank, and from this stack of sheets the desired number of washers may be cut therefrom in a single operation.

20 The washers may then be aligned and fused together as previously set forth. Or, the stack of sheets may be molded together before the cutting operation, and a unitary blank cut from the this slab. In either event, the fiber is cut in a direction perpendicular to the long axis of the threads.

25 The plurality of woven or unwoven cellular or cellulosic or inorganic threads or fibers may be dyed, mercerized or otherwise treated before impregnation, and the impregnating medium may be colored as by addition of dyestuff of pigment.

30 It is to be understood that the foregoing examples and drawings are for illustrative purposes only, and are not to be considered as limitations of the scope of the invention.

35 What I claim is:

1. Process for making a blank comprising impregnating fabric sheets with a thermoplastic body, cutting washer-like members therefrom, aligning the washers along a common axis compacting the washers into a unitary member and roughening the outer surface until ends of fibers protrude therefrom.

40 2. Process for making a roller comprising coating fabric with a thermoplastic resin cutting washer-like members therefrom aligning the washers on a mandrel molding the same into a unit of desired form, then abrading the outer curved surface so there are immovably affixed outwardly-projecting fiber ends.

45 3. Process for making a roll comprising saturating textile with a synthetic resin of the vinol type, cutting washer-like members therefrom aligning the members on a core molding the washers with heat and pressure into a unitary member of shape desired, then roughening the outer surface so there are immovably affixed outwardly-projecting fiber ends.

50 4. Process for making a temple roll comprising coating on one side cotton with a thermoplastic body cutting washer-like members therefrom aligning the washers along a common axis compacting the same into a unit of desired form then abrading the outer surface until ends of fibers protrude therefrom.

55 5. Process for making a blank comprising coating on both sides duck with a thermoplastic resin cutting washer-like members therefrom aligning the members on a mandrel molding the same into a unitary member of shape desired then roughening the outer curved surface until ends of fibers project therefrom.

60 6. Process for making a roller comprising impregnating duck with a synthetic resin of the vinol type cutting washer-like members there-

from aligning the washer members on a core molding said washers by heat and pressure into a unitary-appearing member of surface formed into alternating ridges and grooves arranged in form of a helix then abrading the ridges until there appears immovably affixed, outwardly-projecting, frictionally-gripping fiber ends.

7. Process for making a roll comprising coating non-cellulosic fiber aggregates with a thermoplastic body cutting washer-like members therefrom aligning the washers along a common axis compacting the same into a unitary member of shape desired then roughening the outer surface until ends of fibers protrude outwardly therefrom.

8. Process for making a temple roll comprising saturating non-cellulosic fibers in fabric form

with a thermoplastic resin cutting washer-like members therefrom compacting the same into a unitary-appearing body of desired form then abrading the outer surface until there appears immovably affixed, outwardly projecting, fiber-gripping ends.

9. Process for making a temple roll comprising compacting and fusing together on to a hollow core a plurality of washer-like members of fabric previously impregnated with suitable thermoplastic synthetic resin and molding the plastic composite so as to form helical ridges and grooves, afterwards abrading the ridges to the outwardly-projecting filament ends of the fabric.

15

CHARLES THOMAS DICKEY.